# EUROPEAN PATENT SPECIFICATION

(11) **EP 4 249 135 B1**
(45) Date of publication and mention of the grant of the patent: **18.12.2024**
(21) Application number: 23162916.3
(22) Date of filing: 20.03.2023
(51) Int. Cl.: B05D 1/26, B05D 3/06, B05D 3/12, B05D 7/06, B05D 7/00

(54) **METHOD FOR COATING PANEL EDGES THROUGH VACUUM COATING HEADS**
VERFAHREN ZUM BESCHICHTEN VON PANEELKANTEN DURCH VAKUUMBESCHICHTUNGSKÖPFE.
PROCÉDÉ DE REVÊTEMENT DE BORDS DE PANNEAUX PAR L'INTERMÉDIAIRE DE TÊTES DE REVÊTEMENT SOUS VIDE.

(30) Priority: 23.03.2022 IT 202200005738
(43) Date of publication of application: 27.09.2023
(73) Proprietor: CEFLA SOCIETA' COOPERATIVA, 40026 Imola (BO) (IT)
(72) Inventor: PETRUCCI, Roberto, 61122 Pesaro (IT)
(74) Representative: Del Nero, Susanna

(56) References cited:
- EP-A1- 3 315 210
- DE-A1- 10 100 518
- DE-A1- 102014 107 492
- DE-A1- 102020 125 687
- IT-A1- FI20 090 093
- US-A- 3 967 581
- US-A1- 2021 121 912

## Description

The present invention relates to a method for coating rigid panels made of wood or other materials, like e.g. MDF (Medium Density Fibreboard) wood, fibreboard or other wooden materials, with liquid painting products. In particular, the present invention relates to a method comprising a plurality of successive steps for applying a fluid coating substance, like a painting product, on an external edge of a panel made of a rigid material with different shapes.

Mainly flat panel means a panel wherein two out of three dimensions are much wider than the third dimensions. Typically, the measures of such panels range 100x300x18 mm to 1250x2400x30 mm.

As known, such panels are coated in order to provide them with an aesthetic effect. E.g., in the case of fibreboard panels, i.e. a low-cost material, side coatings are applied so as to cover their uneven surface.

In a known way in the art, such coating is applied through a coating device making use of suction, of the kind comprising a coating head (vacuum coating head) provided with a chamber fed with a liquid painting product to be applied on the wooden panels.

The chamber of each vacuum coating head typically is provided with an opening shaped according to the shape of the transversal section of the panels to be coated. In particular, the opening is counter-shaped to the transversal profile of the panel edge. The opening is placed aligned along a conveying direction of the panel, corresponding to the longitudinal profile of the edge to be coated.

During the conveying of said panel, the panel edge is conveyed near said opening, which supplies the painting product through an output slot for the liquid painting product. Said slot defines a nozzle that at least partially follows the transversal perimeter of the panel edge, at a constant distance so as to lap the whole surface to be coated.

The dispensing slot is adjacent to at least one suction opening, provided for suctioning the liquid painting product, so as to prevent that said painting product can leak out from the coating head.

In this way, the excess liquid painting product, which is not applied on the edge of the conveying panel, is recovered by the suctioning opening and channelled to a reservoir of the liquid painting product.

By adjusting: a) the viscosity of the liquid painting product; b) the flow rate through the dispensing slot; c) the conveying speed of said panel; d) the degree of vacuum provided by the suction recovering excess painting product, the thickness of the painting product applied on said panel is determined.

In addition to the unevenness typical of wooden surfaces, it is known that the use of vacuum suction tends to raise wood fibres, which protrude outside the film of the applied painting product. In order to avoid this drawback, two strategies can be used: a) using a very thick layer of painting product, so as to cover the raised wood fibre; or alternatively b) sanding the coated edge. The first strategy leads to a high and costly consumption of painting product; the second strategy leads to a more complex coating machine, provided with a greater length due to the presence of many sanding groups.

The applicant has been producing machines provided with one or more vacuum coating heads for suction coating for a long time, one of which is e.g. described in EP3315210A1. Said application describes a vacuum coating head comprising a body, at least a top form and at least a lower form.

In the art, there are known also vacuum coating heads made of a plurality of adjacent plates, e.g. from IT102009901728856 of Makor.

In the art, it is known that in edge coating the greatest difficulties are coating Jpull or undercut edges (see Figure 1). In particular, the more complex the surface, the higher the number of sanding groups.

In the art it is known that in order to obtain panels provided with edges having a suitable quality, coating cycles comprising many successive steps must be performed. The traditional coating cycle today performed by the applicant comprises the following steps:
1. sanding of the rough edge;
2. first coating of the edge;
3. first gelling;
4. second coating of the edge;
5. second gelling;
6. third coating of the edge;
7. third gelling;
8. fourth coating of the edge;
9. drying;
10. final sanding (using at least four band sanding groups + two sanding wheels).

A second coating cycle for a finishing of superior quality comprises the following steps:
1. sanding of the rough edge;
2. first coating of the edge;
3. first gelling;
4. second coating of the edge;
5. drying;
6. sanding (using at least four band sanding groups + two sanding wheels)
7. third coating of the edge;
8. third gelling;
9. fourth coating of the edge;
10. fourth gelling;
11. fifth coating of the edge;
12. fifth gelling;
13. sixth coating of the edge;
14. drying;
15. final sanding (using at least four band sanding groups + two sanding wheels).

The number of painting product applications can range one to six (consequently the apparatus comprises one to six vacuum coating heads), depending on the desired quality of the final product.

US20210121912A1 of Louisiana Pacific Corp describes a method for producing engineered-wood fence pickets. The edge-sanding process produces a smooth side surface on the edges, significantly reducing the number of loose fibres and/or strands, and fills in and/or reduces void spaces. The painting of the pickets is performed through spraying.

US3967581A of Edward Irvin Zirbel describes an apparatus for finishing the edge of particleboard, plywood and the like. The finishing is performed by extruding a fast-drying material.

DE102014107492 of MHF GMBH describes a method for smoothing the edges of workpieces which have at least one porous layer. Said method comprises the following steps: conveying the workpieces on a conveyor in a direction parallel to the edge to be smoothed; allowing a continuous carrier strip to pass over deflection rollers at a speed which is synchronous to the conveying speed of the workpieces, such that a contact section of the carrier strip rests on a section of the edge of at least one workpiece to be smoothed over a certain length; applying, upstream of the contact section, a curable filler onto the carrier strip; transferring the filler on the contact section onto the edge such that it forms a continuous layer of predetermined thickness; and allowing the filler to cure, once the carrier strip has been removed, until the continuous layer forms a smooth, solid surface.

DE10100518 of Joseph Schiele OHG describes a device for coating the lateral edge faces of elongate work pieces with a liquid coating medium. The inventive device comprises an adjustable coating head with a coating slot that extends in the direction of transport of the work piece. Said coating head applies the liquid coating medium through just one nozzle at a time.

ITFI20090093 of Makor SRL describes a coating vacuum head for panels comprising a screeding organ placed downstream the organ supplying a coating product, in order to uniformly distribute said coating product and to remove from said panel a portion of the coating medium in excess.

In the art, it is known using painting products comprising photopolymerizing agents activated by ultraviolet (UV) radiations. Such painting products comprise a plurality of monomers that, once activated by UV radiations emitted by lamps of suitable wavelength, are involved in a photopolymerizing process leading to the formation of a polymer network. The quantity of radiation administered to the film of painting product applied on the panel can lead to an incomplete polymerization (gelling) or to a complete polymerization, wherein all the monomers contained in the painting product are concatenated in a polymer network (drying).

The gelling/drying of the painting product can be described in terms of percentage of monomers that react after undergoing UV radiation: indicatively, if complete drying corresponds to about 100% of polymerized monomers, gelling corresponds to about 50% of polymerized monomers after the action of UV radiation. It is intuitive that sanding must occur on a painting product sufficiently polymerized so that it does not stick to sanding groups.

In terms of adjusting the apparatus for coating edges, the percentage of polymerization of the applied painting product depends also on the power of the lamp used for the gelling step. Again indicatively, the polymerizing lamps emitting UV radiations for gelling are set on about 80 W/cm, while for drying the polymerizing lamps are set on about 150 W/cm. It is also worth mentioning that gelling is preferably performed using gallium lamps, while drying is preferably performed using mercury lamps.

The known art coating method is performed through known art apparatuses, which substantially are apparatuses having a given length, in that each of the above-described ten or fifteen steps is performed by a group (sanding group, coating group, gelling group, drying group) placed in series with respect to the preceding and following group. The working of panel edges occurs in passing. Typically, a known art apparatus is 10 to 30 metres long. The length of the apparatus is directly proportional to the number of groups provided in the apparatus, which in turn is directly proportional to the desired quality of the finished panel.

Aim of the present invention is providing a method and an apparatus to perform such method for vacuum coating making use of one or more vacuum coating heads, which is cheaper to perform and that allows to obtain better results in terms of the quality of the coated panel.

This object is achieved by a method and an apparatus having the features of the independent claims. Advantageous embodiments and refinements are specified in claims dependent thereon.

The method according to the present invention provides the following successive steps:
1. sanding of the rough edge;
2. first application of painting product to the edge;
3. first gelling;
4. post-gelling sanding of the edge;
5. second application of painting product to the edge;
6. drying;
7. post-drying sanding.

In an alternative embodiment, for a superior quality of the coated edge, the successive steps are:
1. sanding of the rough edge;
2. first application of painting product to the edge;
3. first gelling;
4. post-gelling sanding of the edge;
5. second application of painting product to the edge;
6. second gelling;
7. third application of painting product to the edge;
8. drying;
9. post-drying sanding.

Substantially, the novelty of the present method with respect to the known art lies in the following two features:
- the application of the painting product occurs through the application of two layers of painting product in a close succession, in a wet-on-wet mode;
- the first sanding after the first application of painting product is performed on the painted product which underwent gelation only, wherein a significant percentage of monomers is not polymerized; obviously, the degree of polymerization must be suitable so that the coated layer can be sanded.

By performing a sanding step after the first application of coating followed by gelling the following results are obtained:
- a smooth surface, because the fibre of the wooden material protruding from the film of painting product is cut (sanded);
- the following applications of painting products are much smoother: the orange peel effect is nearly completely removed, and therefore the final sanding of the panel is easier and requires a lesser number of sanding groups.

The new coating cycle allows to obtain many advantages:
- If instead of gelling it, the applied coating were dried, as oftentimes one must do, the edge should be sanded over its whole coated surface using many sanding groups; while with gelation, only the portion of the edge wherein the wooden fibre is raised is sanded. The sanding on the gelled portion is easier, in that a lesser number of sanding groups are necessary in order to reach all the surfaces of a complex edge like e.g. a Jpull edge: just a sanding wheel or a band are sufficient;
- The following applications of painting products are eased by the lack of protruding wooden fibres; the coating is more efficient, and finally this allows a reduction in the number of steps and of the final thickness of the layers of applied painting product;
- The quantity of energy is markedly reduced (of about 20%, up to 35% according to apparatus configuration).

Experimentally, it was shown that by using a vacuum coating head applying two layers of painting product each according to the new method, the same qualitative result as using two known art vacuum coating heads is obtained.

Experimentally, it was shown that by using three vacuum coating heads applying two layers of painting product each according to the new method, the same qualitative result as using six known art vacuum coating heads is obtained.

Overall, the number of coating heads is reduced, and therefore there is a saving in the number of elements used both for applying and drying the painting product, which allows to reduce the overall length of the apparatus. Experimentally, it was shown that the quality of the finished panel being the same, the new method for applying a painting product allows to produce apparatuses that are 1-5 metres shorter with respect to the currently used apparatuses performing the known art coating cycle, with a significant saving in the required industrial space.

It is worth noting that the number of sanding groups placed downstream the coating groups, affecting the overall length of the apparatus, depends on the geometrical shape of the edge to be sanded and on the quality of the desired finishing.

All this translates into an apparatus that provides a coating of outstanding quality but much cheaper to produce and of shorter length, without considering the savings in terms of energy consumption during the functioning of the apparatus.

Further advantages and properties of the present invention are disclosed in the following description, in which exemplary embodiments of the present invention are explained in detail based on the drawings:
- Figure 1: Examples of panels provided with different edges: undercut edge, Jpull edge, radius edge, in transversal section;
- Figure 2: Known art apparatus provided with four coating heads, top view;
- Figure 3: Apparatus according to the present invention configured for providing four painting product applications, top view;
- Figure 4: Known art apparatus provided with two coating heads and apparatus according to the present invention configured for providing four painting product applications, top view;
- Figure 5: Known art apparatus provided with three coating heads and apparatus according to the present invention configured for providing four painting product applications, top view;
- Figure 6: Known art apparatus provided with five coating heads and apparatus according to the present invention configured for providing four painting product applications, top view;
- Figure 7: Known art apparatus provided with six coating heads and apparatus according to the present invention configured for providing six painting product applications, top view;
- Figure 8A, 8B: Vacuum coating head according to the present invention in front and axonometric view.

For the sake of clarity, in this Description a vacuum tower, indicated in this Description with the numeral 14, means a unit providing both the painting product and the vacuum to the vacuum head.

Figure 1 shows a first mainly flat panel 1 provided with an undercut edge 2, a second mainly flat panel 1' provided with a Jpull edge 3, and a third mainly flat panel 1" provided with a radius edge 4. Said Jpull edges are e.g. used in kitchen cabinet doors, as they allow to open said doors while their external surface is free of handles or doorknobs. Figure 1 is illustrative only, having the aim to show the plurality of different edges that can be coated by a vacuum coating head according to the present invention. There is provided a wide variety of edges that are not shown in Figure 1.

Any panel is provided with two main sides and four edges, each of which must be coated. Panel coating typically occurs in production lines comprising a plurality of apparatuses placed in series. According to the organization of the production line characteristic of each production plant, for coating each side and edge there can be provided a specific apparatus, and between said apparatuses there is provided a turning device allowing to provide the following apparatus with the side or edge to be coated by that specific apparatus. Alternatively, the same apparatus can paint the four edges: the panel is conveyed four times inside the same apparatus. Alternatively, an apparatus according to the present invention coats the geometrically more complex edge, while one or further apparatus/es is/are provided for the coating of the geometrically less complex edges.

In the art, there are known apparatuses provided with variable numbers of post-coating sanding groups. The more geometrically complex the edge 2, 3, 4, the higher the number of sanding groups provided in the apparatus in order to have a perfectly coated panel, in that each of them is adjusted to sand just one portion of said edge. It is worth noting that, according to the kind of batch produced in a given moment, in an apparatus provided with a high number of sanding groups, some sanding groups might be inactive during the production of that specific batch.

In Figure 2 and 3 a known art apparatus 410 with four coating heads according to the known art and an apparatus 430 applying four layers of painting product according to the present invention are compared. This is just one of many possible configurations, some of which are shown in Figures 4-7.

It is worth mentioning that in the following Description, the apparatuses indicated by the numeral 10 preceded by a digit indicate apparatuses according to the known art, while the apparatuses indicated by the numeral 30 preceded by a digit indicate apparatuses according to the present invention. The digit preceding 10 or 30 indicates the number of applications of painting product performed by the apparatus.

Both in the known art apparatuses *10 and in the apparatuses *30 according to the known art, a panel 1 is conveyed by a (not shown) conveying band (chain conveyor) that is narrower than the panel dimension perpendicular to the conveying direction. The panel is cantilevered with respect to the apparatus * 10, *30. Just one edge at a time of the panel 1 is worked during each passage inside the apparatus *10, *30; obviously, the edge undergoing coating is the one adjacent to the apparatus. Panels 1 can be manually uploaded/downloaded in/from the apparatus *10, *30 by a human operator, or loading/unloading can occur automatically using known conveyors. In a known way, apparatuses * 10, *30 are provided with an aligner pushing the panel 1 against a reference stop. Optionally the same apparatus *10, *30 can be used to coat also the other edges of panels 1, one at a time.

As explained above, the length of the apparatus varies proportionally to the numerousness of groups. In this first comparison (Figure 2 and 3) a known art apparatus provided with four coating head according to the known art and an apparatus applying four layers of painting product according to the present invention are compared. The number of sanding groups placed downstream the drying group is the same, so as to show a meaningful comparison in terms of apparatus length between the known art apparatus and an apparatus according to the present invention.

The bold arrows show the conveying direction of the panel 1, whose edges must be coated.

Figure 2 shows a known art apparatus 410 currently produced by the applicant, in a top view.

The known art apparatus 410 comprises:
- a sanding group 11 for a coarse pre-coating sanding;
- a sanding group 12 (here in the shape of a sanding wheel) for a finer sanding;
- four vacuum coating heads 13, 13', 13", 13''';
- two vacuum towers 14, 14'
   each vacuum tower supplies a painting product to two coating heads: in particular, the vacuum tower 14 supplies said painting product to the vacuum heads 13, 13', while the vacuum tower 14' supplies said painting product to the vacuum heads 13", 13‴;
- three gelling groups 15, 15', 15"
   said gelling groups comprise preferably one or more gallium lamps which partially polymerize the monomers of the painting product;
- two drying groups 16, 16'
   said drying groups comprise one or more mercury and/or gallium lamps which completely polymerize the monomers of the painting product;
- a belt sanding group 17;
- four sanding groups 18, 18', 18", 18'" for a coarse post-coating sanding;
- three sanding groups 19, 19', 19" for a finer post-coating sanding (sanding wheels);
- two corner sanding groups 20, 20', for sanding the head and the tail of panel 1, respectively;
- a sanding group 21 for the final sanding: this is a sanding group provided with a belt with a particularly fine grain.

Figure 3 shows an apparatus 430 according to the present invention, in top view.

The apparatus 430 according to the present invention comprises:
- a sanding group 11 for a coarse pre-coating sanding;
- a sanding group 12 (here in the shape of a sanding wheel) for a finer sanding;
- two vacuum coating heads 23, 23';
- one vacuum tower 14;
- two gelling groups 15, 15';
- a sanding group 22 placed immediately downstream the first gelling group 15, 15';
- two drying groups 16, 16';
- a belt sanding group 17;
- four sanding groups 18, 18', 18", 18'" for a coarse post-coating sanding;
- three sanding groups 19, 19', 19" for a finer post-coating sanding (sanding wheels);
- two corner sanding groups 20, 20', for sanding the head and the tail of panel 1, respectively;
- a sanding group 21 for the final sanding: this is a sanding group provided with a belt with a particularly fine grain.

At a glance, it can be observed that the apparatus 430 according to the present invention is shorter than the known art apparatus 410.

Figure 4 compares a known art apparatus 210 provided with two coating heads 13, 13' and an apparatus 430 applying four layers of painting product according to the present invention. In the Figure, just the portions concerning the coating are indicated. As explained above, the portions downstream the coating portion are variable according to the panels to be coated. The downstream portion comprising the sundry sanding groups is purposefully identical in the two apparatuses, so as to facilitate the comparison between the known art apparatus 210 and the apparatus 430 according to the present invention.

In the case of a panel requiring four applications of painting product, with the apparatus 430 according to the present invention, the panel is conveyed just once inside the apparatus. Instead, with the known art apparatus 210, the same panel must be conveyed twice inside the apparatus 210: the apparatus is shorter, but the coating cycle must be repeated in order to obtain a qualitative result comparable to that obtainable with just one cycle in the apparatus 430 according to the present invention.

Figure 5 compares a known art apparatus 310 provided with three coating heads 13, 13', 13" and an apparatus 430 applying four layers of painting product according to the present invention. In the Figure, just the portions concerning the coating are indicated. As explained above, the portions downstream the coating portion are variable according to the panels to be coated. The downstream portion comprising the sundry sanding groups is purposefully identical in the two apparatuses, so as to facilitate the comparison between the known art apparatus 310 and the apparatus 430 according to the present invention.

The result obtained with the apparatus 310 and the apparatus 430 is not equivalent: in fact, with the apparatus 310 three layers of painting product are applied, while with the apparatus 430 four layers of painting product are applied. With a comparable length of the two apparatuses, the qualitative result is better with the apparatus 430. Moreover, with the apparatus 430 a vacuum tower is dispensed with.

Figure 6 compares a known art apparatus 510 provided with five coating heads 13, 13', 13", 13"', 13"" according to the known art and an apparatus 530 applying four layers of painting product according to the present invention. In the Figure, just the portions concerning the coating are indicated. As explained above, the portions downstream the coating portion are variable according to the panels to be coated. The downstream portion comprising the sundry sanding groups is purposefully identical in the two apparatuses, so as to facilitate the comparison between the known art apparatus 510 and the apparatus 530 according to the present invention.

Figure 6 shows a particular embodiment, wherein each vacuum coating head 23, 23' of the apparatus 30 is supplied by a respective vacuum tower 14, 14'. As explained above, a vacuum tower 14 can supply two and even three vacuum coating heads 23, 23'. In this case, though, there are provided two distinct vacuum towers 14, 14': the first vacuum tower supplies a primer to the first vacuum coating head 23, while the second vacuum tower 14' supplies a painting product to the second vacuum coating head 23'.

Figure 7 compares a known art apparatus 610 provided with six coating heads 13, 13', 13", 13‴, 13ʺʺ, 13ʺ‴ according to the known art and an apparatus 630 applying six layers of painting product according to the present invention. In the Figure, just the portions concerning the coating are indicated. As explained above, the portions downstream the coating portion are variable according to the panels to be coated. The downstream portion comprising the sundry sanding groups is purposefully identical in the two apparatuses, so as to facilitate the comparison between the known art apparatus 610 and the apparatus 630 according to the present invention.

In the case of the apparatus 630 applying six layers of painting product, the second gelling step is performed by just one gelling group 15" followed by a third application of painting product performed by a third vacuum coating head 23". Finally, the last gelling/drying step is performed by a gelling/drying group 16, 16'. Of course, this apparatus is used for finishing of a particularly high quality.

Figures 2, 3, 6 and 7 allow to visually appreciate the reduction in the length of the apparatuses according to the present invention with respect to the known art apparatuses, the number of applications of painting product being the same. Said reduction in length can indicatively range 1 to 5 metres.

The method according to the present invention comprises the following steps performed by an apparatus 430:
1. sanding of the rough edge
   performed by the sanding groups 11 and 12 placed upstream the vacuum head 23;
2. first application of painting product to the edge
   performed by the first vacuum coating head 23;
3. gelling
   performed by two gelling groups 15, 15', preferably comprising one or more gallium lamps;
4. post-gelling sanding of the edge
   performed with sanding wheels, bands or any other sanding system by the sanding group 22;
5. second application of painting product to the edge
   performed by the second vacuum coating head 23'; the first vacuum coating head 23 and the second coating head 23' are preferably supplied by just one vacuum tower 14;
6. drying
   performed by the drying group 16, 16', preferably comprising one or more mercury lamps;
7. post-drying final sanding
   performed by a number of sanding groups 17, 18, 19, 20, 21 proportional to the desired quality of the finished panel.

In an alternative embodiment, suitable for a superior quality of the coated edge, the method according to the present invention comprises the following steps performed by an apparatus 630:
1. sanding of the rough edge
   performed by the sanding groups 11 and 12 placed upstream the vacuum head 23;
2. first application of painting product to the edge
   performed by the first vacuum coating head 23;
3. first gelling
   performed by at least one, preferably two gelling groups 15, 15';
4. post-gelling sanding of the edge
   performed with sanding wheels, bands or any other sanding system by the sanding group 22;
5. second application of painting product to the edge
   performed by the second vacuum coating head 23';
6. second gelling
   performed by at least one gelling groups 15";
7. third application of painting product to the edge
   performed by the third vacuum coating head 23";
8. drying
   performed by the drying group 16, 16';
9. post-drying final sanding
   performed by a number of sanding groups 17, 18, 19, 20, 21 proportional to the desired quality of the finished panel.

It is worth mentioning that in the apparatuses *30 according to the present invention, the gallium lamp in the gelling group 15, 15' are set on 80 W/cm, the gallium lamps in the gelling group 16 are set on 60-65 W/cm, while the mercury lamps in the drying group 16' are set on 120-150 W/cm. These power levels, too, contribute to the reduced energy consumption with respect to the known art apparatuses.

Alternatively, in lieu of the gallium and mercury lamps, LED lamps ranging 8 W up to 20 W can be used. In this case, indicatively, for gelling steps 20 W LED lamps are set on 10-12 W/cm², while for drying steps 20 W LED lamps are set on 18-20 W/cm².

The sanding group 22 is preferably provided in the form of a sanding wheel with a cloth Trizact^{©} 3M^{®}, comprising a ceramic abrasive material supported by a polyester cloth.

The sanding performed by the sanding group 22, placed between the application of the first two layers of painting product applied by the first vacuum coating head 23, and the application of the second two layers of painting product applied by the second vacuum head 23', allows to obtain a coated surface that is smoother and more even. Consequently, with the following applications of painting product an even better result is obtained. The final sanding performed with the sanding groups downstream the second vacuum coating head 23' allows to obtain a perfectly smooth surface.

Figures 8A, 8B show a vacuum head 23 that is advantageously comprised inside the apparatuses *30 according to the present invention. Said vacuum head allows to maximize the advantages applying the method according to the present invention.

Said vacuum coating head 23 comprises:
- a pair of bores 50 for fixing said head to a support allowing to connect said head to the apparatus 430;
- a first dispensing nozzle 51 for dispensing a painting product;
- a first suction nozzle 52 for suctioning said painting product;
- an optional screed 53;
- a second dispensing nozzle 55 for dispensing said painting product;
- a second suction nozzle 56 for suctioning said painting product.

In the preferred embodiment, between the first suction nozzle 52 for suctioning a painting product and the second dispensing nozzle 55 for dispensing a painting product, there is provided a screed 53 protruding with respect to the profile of the vacuum coating head for a length ranging 0,1 to 0,5 mm. This minimal protrusion, difficult to be appreciated in the Figures, allows the screed 53 to perform two actions:
- pressing the applied painting product inside wood pores;
- pressing the wooden fibres raised by the suction generated by the first suction nozzle 52.

Here is worth noting that up to the introduction of 3D printing the vacuum coating heads used to be produced in the form of coating heads made of a plurality of plates, as in this way obtaining cavities in solid pieces used to be easier. It is known obtaining said plates in metallic materials, in a plastic material, or even in a wooden material (phenolic wood).

Nowadays, with 3D printing, pieces provided with internal cavities can be produced through additive manufacturing; therefore, the vacuum head 23 according to the present invention can be produced in a single solid piece, produced in plastic material, e.g. in epoxy resin, or in a metallic material, e.g. aluminium or stainless steel, provided with suitable characteristics.

It is worth noting that the vacuum coating head 23, provided with two dispensing nozzles 51, 55 in fact applies two layers of painting product with respect to the vacuum known art coating head 13, which is provided with just one dispensing nozzle. The application of painting product by the second dispensing nozzle 55 on the first layer of painting product dispensed by the first dispensing nozzle 51 is in fact a wet-on-wet application, as the gelling group 15 is placed downstream each vacuum coating head 23.

The skilled man has the entrenched prejudice that by gelling the applied layer before applying the second layer of painting product a better result will be obtained, due to the better adhesion of the successive layer of painting product on a dried or at least gelled layer. Surprisingly, it was observed that the presence of the screed compensates for the lack of gelation, and it presses the wood fibres raised by the first suction nozzle 52. This overall allows to provide a higher quantity of painting product on the panel 1 with respect to the usual coating method (application of painting product - gelation - successive application of painting product).
- 1: panel
- 2: undercut edge
- 3: Jpull edge
- 4: radius edge
- 11: coarse sanding group
- 12: sanding group
- 13: vacuum coating head
- 14: vacuum tower
- 15: gelling group
- 16: drying group
- 17: band sanding group
- 18: coarse sanding group
- 19: fine sanding group
- 20: corner sanding group
- 21: final sanding group
- 22: sanding group
- 23: vacuum coating head
- 50: bore
- 51: first dispensing nozzle
- 52: first suction nozzle
- 53: screed
- 55: second dispensing nozzle
- 56: second suction nozzle
- 57: bore
- 58: bore
- 210: known art apparatus with two coating heads
- 310: known art apparatus with three coating heads
- 410: known art apparatus with four coating heads
- 430: apparatus according to the present invention with four applications of painting product
- 510: known art apparatus with five coating heads
- 530: apparatus according to the present invention with four applications of painting product
- 610: known art apparatus with six coating heads
- 630: apparatus according to the present invention with six applications of painting product

## Claims

1. Method for applying a painting product, preferably an UV painting product, to an edge of wooden panels (1) through an apparatus comprising pre-coating sanding groups (11, 12) and post-drying sanding groups (17, 18, 19, 20, 21), at least a painting group provided in the form of a vacuum coating head (23) supplied with both said painting product and vacuum by a vacuum tower (14), at least a gelling group (15), at least a drying group (16) placed in series comprising the following successive steps:
1. sanding of the rough edge;
2. first application of painting product to the edge;
3. first gelling;
4. post-gelling sanding of the edge;
5. second application of said painting product to the edge;
6. drying;
7. final post-drying sanding;
**characterized in that**
- in each one of steps 2 and 5, the application of said painting product to the panel edge occurs through two layers of painting product applied in a wet-on-wet close succession;
- in step 4, the post-gelling sanding occurs on a layer of painting product that underwent gelation only.

2. Method for applying a painting product, preferably an UV painting product, to an edge of wooden panels (1) through a vacuum coating head (23) according to claim 1, wherein for a superior quality of the finished panel a further application of painting product is provided, according to the following successive steps:
1. sanding of the rough edge;
2. first application of painting product to the edge;
3. first gelling;
4. post-gelling sanding of the edge;
5. second application of painting product to the edge;
6. second gelling;
7. third application of painting product to the edge;
8. drying;
9. post-drying sanding.

3. Method for applying a painting product, preferably an UV painting product, to an edge of wooden panels (1) through a vacuum coating head (23) according to claim 1 or 2, wherein said wet-on-wet applications of painting product occurs through a vacuum coating head (23) provided at least with two nozzles (51, 55) for applying said painting product.

4. Apparatus (430, 530, 630) for performing the method according to claims 1-3 for applying a painting product, preferably an UV painting product, to an edge of wooden panels (1), said apparatus comprising in that order:
1. first sanding groups (11, 12) placed upstream the first vacuum head (23);
2. first coating head (23) for applying a painting product to the panel edge, applying two wet on wet layers of the painting product in a close succession;
3. at least one, preferably two gelling groups (15, 15'), preferably comprising one or more gallium lamps;
4. post-gelling sanding group (22) of the edge, preferably in the form of sanding wheels, bands;
5. second vacuum coating head (23') for applying a painting product to the edge, applying two wet on wet layers of the painting product in a close succession:
6. at least a drying group (16, 16');
7. post-drying final sanding groups (17, 18, 19, 20, 21) in a number proportional to the desired quality of the finished panel.

5. Apparatus (630) for applying a painting product, preferably an UV painting product, to an edge of wooden panels (1) according to claim 4 comprising in that order:
1. first sanding groups (11, 12) placed upstream the first vacuum head (23);
2. first vacuum coating head (23) for applying a painting product to the panel edge, applying two wet on wet layers of the painting product in a close succession;
3. at least one first, preferably two gelling groups (15, 15');
4. post-gelling sanding group (22), preferably in the form of sanding wheels, bands;
5. second vacuum coating head (23') for applying a painting product to the panel edge, applying two wet on wet layers of the painting product in a close succession;
6. at least one second gelling group (15");
7. third vacuum coating head (23") for applying a painting product to the panel edge, applying two wet on wet layers of the painting product in a close succession;
8. at least a drying group (16, 16');
9. post-drying final sanding groups (17, 18, 19, 20, 21) in a number proportional to the desired quality of the finished panel.

6. Apparatus (430, 530, 630) according to claim 4 or 5, wherein each vacuum tower (14) supplies one, preferably two or three vacuum coating heads (23, 23', 23").

7. Apparatus (430, 530, 630) according to one or more of claims 4-6, wherein when the painting products to be applied to an edge are more than one, there is provided a number of vacuum towers (14) equal to the number of painting products used in the coating process.

8. Apparatus (430, 530, 630) according to one or more of claims 4-7, wherein the lamps in said gelling groups (15) are gallium lamps, preferably set at 60-80 W/cm, or LED lamps preferably set at 10-12 W/cm².

9. Apparatus (430, 530, 630) according to one or more of claims 4-7, wherein the lamps in said drying groups (16, 16') are gallium lamps or mercury lamps preferably set at 120-150 W/cm or alternatively LED lamps preferably set at 18-20 W/cm².

## Patentansprüche

1. Verfahren zum Auftragen eines Anstrichprodukts, vorzugsweise eines UV-Anstrichprodukts, auf eine Kante von Holzplatten (1) mittels einer Vorrichtung, die Folgendes aufweist: Vorbeschichtungs-Schleifgruppen (11, 12) und Nachtrocknungs-Schleifgruppen (17, 18, 19, 20, 21), mindestens eine Anstrichgruppe, die in Form eines Vakuumbeschichtungskopfes (23) vorgesehen ist, der von einem Vakuumturm (14) sowohl mit dem Anstrichprodukt als auch mit Vakuum versorgt wird, mindestens eine Geliergruppe (15) und mindestens eine Trocknungsgruppe (16), die in Reihe angeordnet sind, wobei das Verfahren die folgenden aufeinanderfolgenden Schritte umfasst:
1. Schleifen der rauen Kante;
2. erstes Auftragen von Anstrichprodukt auf die Kante;
3. erstes Gelieren;
4. Schleifen der Kante nach dem Gelieren;
5. zweites Auftragen des Anstrichprodukts auf die Kante;
6. Trocknen;
7. abschließendes Schleifen nach dem Trocknen;
**dadurch gekennzeichnet, dass**
- in jedem der Schritte 2 und 5 das Auftragen des Anstrichprodukts auf die Plattenkante durch zwei Schichten Anstrichprodukt erfolgt, die in dichter Folge Nass-in-Nass aufgetragen werden;
- in Schritt 4 das Schleifen nach dem Gelieren auf einer Schicht des Anstrichprodukts erfolgt, die nur Gelierung unterzogen worden ist.

2. Verfahren zum Auftragen eines Anstrichprodukts, vorzugsweise eines UV-Anstrichprodukts, auf eine Kante von Holzplatten (1) durch einen Vakuumbeschichtungskopf (23) gemäß Anspruch 1, wobei für eine höhere Qualität der fertigen Platte ein weiteres Auftragen von Anstrichprodukt vorgesehen ist, gemäß den folgenden aufeinanderfolgenden Schritten:
1. Schleifen der rauen Kante;
2. erstes Auftragen von Anstrichprodukt auf die Kante;
3. erstes Gelieren;
4. Schleifen der Kante nach dem Gelieren;
5. zweites Auftragen von Anstrichprodukt auf die Kante;
6. zweites Gelieren;
7. drittes Auftragen von Anstrichprodukt auf die Kante;
8. Trocknen;
9. Schleifen nach dem Trocknen.

3. Verfahren zum Auftragen eines Anstrichprodukts, vorzugsweise eines UV-Anstrichprodukts, auf eine Kante von Holzplatten (1) durch einen Vakuumbeschichtungskopf (23) gemäß Anspruch 1 oder 2, wobei das Nass-in-Nass-Auftragen von Anstrichprodukt durch einen Vakuumbeschichtungskopf (23) erfolgt, der mindestens mit zwei Düsen (51, 55) zum Auftragen des Anstrichprodukts versehen ist.

4. Vorrichtung (430, 530, 630) zum Ausführen des Verfahrens nach den Ansprüchen 1 bis 3 zum Auftragen eines Anstrichprodukts, vorzugsweise eines UV-Anstrichprodukts, auf eine Kante von Holzplatten (1), wobei die Vorrichtung in der genannten Reihenfolge aufweist:
1. erste Schleifgruppen (11, 12), die stromaufwärts von dem ersten Vakuumkopf (23) angeordnet sind;
2. einen ersten Beschichtungskopf (23) zum Auftragen eines Anstrichprodukts auf die Plattenkante, wobei zwei Nass-in-Nass-Schichten des Anstrichprodukts in dichter Folge aufgetragen werden;
3. mindestens eine, vorzugsweise zwei Geliergruppen (15, 15'), die vorzugsweise eine oder mehrere Galliumlampen aufweisen;
4. eine Schleifgruppe (22) zum Schleifen der Kante nach dem Gelieren, vorzugsweise in Form von Schleifrädern/Schleifbändern;
5. einen zweiten Vakuumbeschichtungskopf (23') zum Auftragen eines Anstrichprodukts auf die Kante, wobei zwei Nass-in-Nass-Schichten des Anstrichprodukts in dichter Folge aufgetragen werden;
6. mindestens eine Trocknungsgruppe (16, 16');
7. nach der Trocknung verwendete Endschleifgruppen (17, 18, 19, 20, 21) in einer Anzahl proportional zu der gewünschten Qualität der fertigen Platte.

5. Vorrichtung (630) zum Auftragen eines Anstrichprodukts, vorzugsweise eines UV-Anstrichprodukts, auf eine Kante von Holzplatten (1) nach Anspruch 4, die in der genannten Reihenfolge Folgendes aufweist:
1. erste Schleifgruppen (11, 12), die stromaufwärts von dem ersten Vakuumkopf (23) angeordnet sind;
2. einen ersten Vakuumbeschichtungskopf (23) zum Auftragen eines Anstrichprodukts auf die Plattenkante, wobei zwei Nass-in-Nass-Schichten des Anstrichprodukts in dichter Folge aufgetragen werden;
3. mindestens eine erste, vorzugsweise zwei Geliergruppen (15, 15');
4. eine Nachgelier-Schleifgruppe (22), vorzugsweise in Form von Schleifrädern/Schleifbändern;
5. einen zweiten Vakuumbeschichtungskopf (23') zum Auftragen eines Anstrichprodukts auf die Plattenkante, wobei zwei Nass-in-Nass-Schichten des Anstrichprodukts in dichter Folge aufgetragen werden;
6. mindestens eine zweite Geliergruppe (15");
7. einen dritten Vakuumbeschichtungskopf (23") zum Auftragen eines Anstrichprodukts auf die Plattenkante, wobei zwei Nass-in-Nass-Schichten des Anstrichprodukts in dichter Folge aufgetragen werden;
8. mindestens eine Trocknungsgruppe (16, 16');
9. nach der Trocknung verwendete Endschleifgruppen (17, 18, 19, 20, 21) in einer Anzahl proportional zu der gewünschten Qualität der fertigen Platte.

6. Vorrichtung (430, 530, 630) nach Anspruch 4 oder 5,
wobei jeder Vakuumturm (14) einen, vorzugsweise zwei oder drei Vakuumbeschichtungsköpfe (23, 23', 23") speist.

7. Vorrichtung (430, 530, 630) nach einem oder mehreren der Ansprüche 4 bis 6,
wobei dann, wenn mehr als ein Anstrichprodukt auf eine Kante aufzutragen ist, eine Anzahl von Vakuumtürmen (14) vorgesehen ist, die der Anzahl der in dem Beschichtungsprozess verwendeten Anstrichprodukte entspricht.

8. Vorrichtung (430, 530, 630) nach einem oder mehreren der Ansprüche 4 bis 7,
wobei die Lampen in den Geliergruppen (15) Galliumlampen, die vorzugsweise auf 60-80 W/cm eingestellt sind, oder LED-Lampen sind, die vorzugsweise auf 10-12 W/cm² eingestellt sind.

9. Vorrichtung (430, 530, 630) nach einem oder mehreren der Ansprüche 4 bis 7,
wobei die Lampen in den Trocknungsgruppen (16, 16') Galliumlampen oder Quecksilberlampen sind, die vorzugsweise auf 120-150 W/cm eingestellt sind, oder alternativ LED-Lampen sind, die vorzugsweise auf 18-20 W/cm² eingestellt sind.

## Revendications

1. Procédé pour appliquer un produit de peinture, de préférence un produit de peinture UV, sur un bord de panneaux de bois (1) par l'intermédiaire d'un appareil comprenant des groupes de ponçage pré-revêtement (11, 12) et des groupes de ponçage post-séchage (17, 18, 19, 20, 21), au moins un groupe de peinture disposé sous la forme d'une tête de revêtement sous vide (23) alimentée en à la fois ledit produit de peinture et du vide par une tour sous vide (14), au moins un groupe de gélification (15), au moins un groupe de séchage (16), placés en série, comprenant les étapes successives suivantes :
1. ponçage du bord grossier ;
2. première application de produit de peinture sur le bord ;
3. première gélification ;
4. ponçage post-gélification du bord ;
5. deuxième application dudit produit de peinture sur le bord ;
6. séchage ;
7. ponçage post-séchage final ;
**caractérisé en ce que**
- dans chacune des étapes 2 et 5, l'application dudit produit de peinture sur le bord de panneau a lieu par l'intermédiaire de deux couches de produit de peinture appliquées en succession rapprochée humide sur humide ;
- dans l'étape 4, le ponçage post-gélification a lieu sur une couche de produit de peinture qui a subi une gélification uniquement.

2. Procédé pour appliquer un produit de peinture, de préférence un produit de peinture UV, sur un bord de panneaux de bois (1) par l'intermédiaire d'une tête de revêtement sous vide (23) selon la revendication 1, dans lequel, pour une qualité supérieure du panneau fini, une autre application de produit de peinture est prévue, conformément aux étapes successives suivantes :
1. ponçage du bord grossier ;
2. première application de produit de peinture sur le bord ;
3. première gélification ;
4. sablage post-gélification du bord ;
5. deuxième application de produit de peinture sur le bord ;
6. deuxième gélification ;
7. troisième application de produit de peinture sur le bord ;
8. séchage ;
9. ponçage post-séchage.

3. Procédé pour appliquer un produit de peinture, de préférence un produit de peinture UV, sur un bord de panneaux de bois (1) par l'intermédiaire d'une tête de revêtement sous vide (23) selon la revendication 1 ou 2, dans lequel lesdites applications humide sur humide du produit de peinture sont effectuées par l'intermédiaire d'une tête de revêtement sous vide (23) dotée d'au moins deux buses (51, 55) pour l'application dudit produit de peinture.

4. Appareil (430, 530, 630) pour la mise en oeuvre du procédé selon l'une quelconque des revendications 1 à 3 pour appliquer un produit de peinture, de préférence un produit de peinture UV, sur un bord de panneaux de bois (1), ledit appareil comprenant, dans cet ordre :
1. des premiers groupes de ponçage (11, 12) placés en amont de la première tête sous vide (23) ;
2. une première tête de revêtement (23) pour appliquer un produit de peinture sur le bord de panneau, appliquer deux couches humide sur humide du produit de peinture en succession rapprochée ;
3. au moins un, de préférence deux groupes de gélification (15, 15'), de préférence comprenant une ou plusieurs lampes au gallium ;
4. un groupe de ponçage post-gélification (22) du bord, de préférence sous la forme de bandes, de roues de ponçage ;
5. une deuxième tête de revêtement sous vide (23') pour appliquer un produit de peinture sur le bord, appliquer deux couches humide sur humide du produit de peinture en succession rapprochée ;
6. au moins un groupe de séchage (16, 16') ;
7. des groupes de ponçage final post-séchage (17, 18, 19, 20, 21) en un nombre proportionnel à la qualité souhaitée du panneau fini.

5. Appareil (630) pour appliquer un produit de peinture, de préférence un produit de peinture UV, sur un bord de panneaux de bois (1), selon la revendication 4, comprenant dans cet ordre :
1. des premiers groupes de ponçage (11, 12) placés en amont de la première tête sous vide (23) ;
2. une première tête de revêtement sous vide (23) pour appliquer un produit de peinture sur le bord de panneau, appliquer deux couches humide sur humide du produit de peinture en succession rapprochée ;
3. au moins un, de préférence deux groupes de gélification (15, 15') ;
4. un groupe de ponçage post-gélification (22), de préférence sous la forme de bandes, de roues de ponçage ;
5. une deuxième tête de revêtement sous vide (23') pour appliquer un produit de peinture sur le bord, appliquer deux couches humide sur humide du produit de peinture en succession rapprochée ;
6. au moins un deuxième groupe de gélification (15") ;
7. une troisième tête de revêtement sous vide (23") pour appliquer un produit de peinture sur le bord de panneau, appliquer deux couches humide sur humide du produit de peinture en succession rapprochée ;
8. au moins un groupe de séchage (16, 16') ;
9. des groupes de ponçage final post-séchage (17, 18, 19, 20, 21) en un nombre proportionnel à la qualité souhaitée du panneau fini.

6. Appareil (430, 530, 630) selon la revendication 4 ou 5, dans lequel chaque tour sous vide (14) alimente une, de préférence deux ou trois têtes de revêtement sous vide (23, 23', 23").

7. Appareil (430, 530, 630) selon une ou plusieurs des revendications 4 à 6, dans lequel, quand les produits de peinture devant être appliqués à un bord sont plus d'un, il est fourni un nombre de tours sous vide (14) égal au nombre de produits de peinture utilisés dans le procédé de revêtement.

8. Appareil (430, 530, 630) selon une ou plusieurs des revendications 4 à 7, dans lequel les lampes dans lesdits groupes de gélification (15) sont des lampes au gallium, de préférence réglées à 60-80 W/cm, ou des lampes à DEL de préférence réglées à 10-12 W/cm².

9. Appareil (430, 530, 630) selon une ou plusieurs des revendications 4 à 7, dans lequel les lampes dans lesdits groupes de séchage (16, 16') sont des lampes au gallium ou des lampes au mercure de préférence réglées à 120-150 W/cm ou en variante des lampes à DEL de préférence réglées à 18-20 W/cm².
